

## UNITED STATES PATENT OFFICE.

ED HAMBLIN, JR., OF WOODWARD, OKLAHOMA.

## COMPOSITION OF MATTER FOR USE IN THE TREATMENT OF FABRICS.

No Drawing.

Application filed July 23, 1925. Serial No. 45,720.

*To all whom it may concern:*

Be it known that I, Ed HAMBLIN, Jr., a citizen of the United States, residing at Woodward, in the county of Woodward and 5 State of Oklahoma, have invented a new and useful Composition of Matter for Use in the Treatment of Fabrics, of which the following is a specification.

This invention relates to a composition of 10 matter designed primarily for use in the treatment of cloth such as used on the rails of pool tables and billiard tables.

It is a well-known fact that the cloth on 15 the rails soon becomes worn because of the impact of balls thereagainst at certain points. This is particularly true at the sides of the openings to the pockets of pool tables and at the corners of billiard tables.

It is an object of the present invention to 20 provide a preparation which can be applied to the fabric at the points where it is subjected to the greatest wear, this preparation serving to strengthen the fabric so that it can resist wear and prolong the life of the 25 cloth.

Another object is to provide a composition 30 of matter of this type which can be easily applied to the cloth and, when applied, will not interfere with the rebounding of balls propelled thereagainst.

With the foregoing and other objects in view which will appear as the description proceeds, the invention consists of two mixtures which, after being brought together 35 can be applied with an ordinary paint brush to those parts of the fabric to be protected. The first of these mixtures consists of the following ingredients substantially in the proportions stated, to wit:

|                                             | Per cent by volume. |
|---------------------------------------------|---------------------|
| A volatile thinner (turpentine or the like) | 75                  |
| Varnish resin                               | 15                  |
| Aluminum resinate                           | 10                  |

The second mixture consists of the following ingredients substantially in the proportions stated, to wit:

|            | Per cent by volume. |
|------------|---------------------|
| Shellac    | 33 1/3              |
| Glue       | 33 1/3              |
| Banana oil | 50                  |

Eighty-six and two-thirds percent of the first mixture are combined with thirteen and one-third percent of the second mixture and after these ingredients have been thoroughly stirred the preparation can be applied to the cloth at those points where it is to be protected, an ordinary paint brush being used for this purpose. The preparation will dry quickly and will impart to the cloth a wear resisting quality which will prolong the life of the cloth several times. Thus the cost of maintaining pool tables and billiard tables is materially reduced.

What is claimed is:

1. A composition of matter for use in the treatment of the rail fabric of pool tables and the like, including a mixture of varnish resin and aluminum resinate with a volatile thinner and another mixture of 70 glue, shellac and banana oil, approximately 86 2/3 percent of the first mixture being combined with 13 1/3 percent of the second mixture.

2. A composition of matter for use in the treatment of the rail fabric of pool tables and the like, including a mixture of substantially 75 15% of varnish resin, 10% of aluminum resinate, and 75% of a volatile thinner, substantially 86 2/3 percent of this 80 mixture being combined with 13 1/3% of a mixture comprising glue, 33 1/3%, shellac 33 1/3% and banana oil 33 1/3%.

In testimony that I claim the foregoing as my own, I have hereto affixed my signature.

ED HAMBLIN, JR.